

## UNITED STATES PATENT OFFICE

LUDWIG ROSENSTEIN, OF SAN FRANCISCO, CALIFORNIA, ASSIGNOR TO SHELL DEVELOPMENT COMPANY, OF SAN FRANCISCO, CALIFORNIA, A CORPORATION OF DELAWARE

## TERTIARY XANTHATE FLOTATION PROCESS

No Drawing.

Application filed February 1, 1932. Serial No. 590,322.

My invention relates to the flotation of ores, more particularly to the use in the froth flotation of copper, zinc, lead and similar ores, or certain new reagents which increase 5 the efficiency of the flotation operation.

There have been used in the past a number of reagents, which, added in small amounts to a pulp in a flotation circuit, aided in and caused the floating of the mineral 10 particles in a froth, which was then removed and the mineral recovered therefrom. Among such reagents was potassium ethyl 15 xanthate. This reagent has been in extensive use and has been considered highly effective in the flotation of ores, and has been a standard of comparison for reagents.

Flotation effects may be obtained by the use of other xanthates, specifically those of the tertiary xanthate type as denoted by 20 the structural formula



wherein R represents an organic radical containing 25 a carbon atom bonded to the oxygen atom as well as to three other carbon atoms, and wherein M represents an alkali-metal.

The sodium and potassium salts of these xanthates are the ones most preferred and 30 the salts of tertiary-butyl, tertiary-amyl and tertiary-hexyl xanthic acids as well as the higher members of the tertiary-hydrocarbon class may be employed with effect in the flotation art.

These new compounds may be prepared in any desired manner as, for example, by the process described in my U. S. Patent 1,854,525 based on my copending application, Serial 40 No. 406,513, filed November 11, 1929, of which this case is a continuation in part. The collectors may be utilized with any of the well-known accessory reagents such as depressors, regulators, frothers and activators. The tertiary xanthates permit operation in an alkaline medium and are preferably added in the 45 form of a solution.

The particular amount of collector to be added to the flotation machine is dependent upon the character of the ore undergoing 50 treatment; the mineral content of the same,

the hydrogen-ion concentration of the liquid; the tendency of the gangue materials to be carried along with the froth, etc. The quantity of collector to be introduced is at best dependent upon the specific operation and no 55 definite limits can be set down. The addition of .10 lb. or less of tertiary xanthates per ton of pulp should normally be sufficient. The tertiary xanthates may be used alone or together with other collectors, including the use 60 of two or more tertiary xanthates.

In practice, the reagents are added almost automatically although frequent checks are made of the mineral content in the concentrate and the tailings as a guide to the 65 amounts required. If, as is often necessary, a series of flotation machines is used, the different units may vary somewhat in the proportion of reagents added. This is especially 70 true when two minerals are to be selectively separated from the gangue.

The degree of fineness to which the ore is originally ground is very important, although in many instances discarded tailings from previous mining operations are ideally 75 suited to reworking by my flotation process.

The expression "tertiary xanthic acid" embraces compounds of the structural formula



wherein R represents an organic radical containing a carbon atom which is bonded to the oxygen atom as well as to three other carbon atoms.

I claim as my invention:

1. A method of recovering minerals from ores which comprises: subjecting an ore to a froth flotation operation in the presence of a salt of a tertiary xanthic acid as a promoter. 90

2. A method of recovering minerals from ores which comprises: subjecting an ore to a froth flotation operation in the presence of an alkali-metal salt of a tertiary xanthic acid as a promoter. 95

3. A method of recovering minerals from ores which comprises: subjecting an ore to a froth flotation operation in the presence of the sodium salt of a tertiary xanthic acid as a promoter. 100

4. A method of recovering minerals from ores which comprises: subjecting an ore to a froth flotation operation in the presence of a compound of the structural formula

5



wherein M represents an alkali-metal as a promoter.

5. A method of recovering minerals from ores which comprises: subjecting an ore to a froth flotation operation in the presence of the sodium salt of tertiary butyl xanthic acid as a promoter.

6. A method of recovering minerals from ores which comprises: subjecting an ore to a froth flotation operation in the presence of an alkali-metal salt of tertiary amyl xanthic acid as a promoter.

7. A method of recovering minerals from ores which comprises: subjecting an ore to a froth flotation operation in the presence of the sodium salt of tertiary amyl xanthic acid as a promoter.

In testimony whereof, I have hereunto set my hand.

LUDWIG ROSENSTEIN.

30

35

40

45

50

55

60

65